

# United States Patent Office

2,731,358

Patented Jan. 17, 1956

1

2,731,358

## PLASTIC FLOOR COVERINGS AND METHOD FOR PRODUCING SAME

James E. Hazeltine, Jr., Lancaster, Pa., assignor to Armstrong Cork Company, Lancaster, Pa., a corporation of Pennsylvania

No Drawing. Application November 10, 1952,  
Serial No. 319,795

4 Claims. (Cl. 117—15)

This invention relates to plastic floor coverings. More particularly, the invention relates to a plastic floor covering obtained by depositing a film of plastic onto a seal-coated saturated felt backing and heating the resulting materials to produce a felt base floor covering characterized by resilience, flexibility, and resistance to alkalies and oils normally employed in the home.

Felt base floor coverings are well known to the art and, generally speaking, they comprise a saturated felt backing, a seal coat, and a paint film which serves as both a decorative and a wearing surface. One widely used method of producing such floor coverings involves the steps of face coating a saturated felt sheet with a coating paint by means of a knife or other suitable apparatus to provide what is known in the art as a seal coat. Following the application of the seal coat, the material is passed through a block printing apparatus. The blocks are dipped into a container of decorative material and various designs are applied by means of the blocks to the coated felt base. Following the application of the decorative coating, the material is dried to produce a hard paint film.

Various coatings have been used for decorating the surface of a seal-coated saturated felt. Generally speaking, these coatings have been what are known to the art as print paints which contain the desired color pigments and a drying oil-resin type vehicle. These drying oil-resin type vehicles have found wide use in the production of printed felt base goods, but it has been difficult to attain the desired alkali resistance in such a floor covering because of the nature of the decorative wearing surface coating.

Recently there have been developed methods of producing a type of printed felt base floor covering in which the more recently developed synthetic plastics have been employed as the wearing surface coat. These synthetic plastics, such as the vinyl resins, for example, copolymers of vinyl chloride and vinyl acetate, polymers of vinyl chloride, and the like, possess outstanding wearing characteristics and are highly resistant to alkalies and washing powders which have had a rather adverse effect on the drying oil type vehicles.

In order to produce attractive patterns of plastic floor coverings by the block printing method, it has been necessary to utilize organosols and plastisols having viscosities within particular ranges. This has been necessary to obtain proper leveling of the paint after application by the printing block. A typical organosol print paint binder contains a plasticizer such as dioctyl phthalate, a polyvinyl chloride resin, and a solvent such as mineral spirits. To this binder is added the pigment, which may be any of the pigments well known in the art, such as titanium dioxide, lead chromate, and the like. In the production of printed organosol floor coverings, the material after printing is heated to fuse the vinyl resin coating. While the floor coverings obtained by such a process exhibit outstanding characteristics, it has been found that such floor coverings are subject to gouging, which may occur during the life of the floor covering when furniture is moved or other

2

objects are moved over the surface of the floor covering.

I have found that this undesirable property is due to the solvent action of the plasticizers, solvents, and diluents employed in the organosol formulation on the coating paints which have been normally used in the production of printed felt base floor coverings. I have further found that this may be overcome by the addition of an aqueous solution of casein to the felt base coating paint. Therefore, in its broadest aspect, my invention may be said to relate to a floor covering obtained by printing a vinyl resin formulation onto a coated felt base in which the coating paint binder contains casein. In a particularly advantageous embodiment of my invention, the coating paint binder contains about 3% to about 20% casein on a dry basis. When less than about 3% casein is present in the binder, there is no significant improvement in gouge resistance of the finished floor covering. When more than about 20% casein is present, the finished floor covering is too stiff. Such floor coverings are then heated, advantageously at about 290° F. to about 350° F., to fuse the print paint and to produce a product having a hard top coat which exhibits improved resistance to indentation and gouging.

In accordance with my invention, the backing material is a sheet of saturated felt which is advantageously one obtained by saturating felt with asphalt, synthetic resin, synthetic rubber, or other material. It is advantageous to utilize a waterproof felt such as one produced by saturation with asphalt, but it is also within the scope of my invention to employ a felt which is saturated with materials which are not highly resistant to the action of water.

To the saturated felt backing a coating paint having a binder containing casein is applied. A typical formulation is illustrated by the following example:

| Example I                               |  | Parts by weight |
|-----------------------------------------|--|-----------------|
| Emulsified oleoresinous varnish         |  | 2520            |
| Casein solution                         |  | 1200            |
| Red slate flour                         |  | 5615            |
| 30 Barden clay                          |  | 890             |
| Water                                   |  | 1700            |
| Concentrated ammonia (aqueous solution) |  | 18              |
| Caustic soda                            |  | 16              |

The casein solution may be prepared in a number of ways, and a typical formulation of such solution is as follows:

| Example II                              |  | Parts by weight |
|-----------------------------------------|--|-----------------|
| Caesin                                  |  | 110             |
| 50 Water                                |  | 576             |
| Concentrated ammonia (aqueous solution) |  | 26              |
| Sodium fluoride                         |  | 2.5             |

This coating paint may be applied by means of a doctor blade or any conventional coating means; and after application, the coated felt is passed through the block printing apparatus. The desired pattern is printed onto the coated felt and the print paint may comprise any of the organosol print paints known to the art, a typical example being as follows:

| Example III                                                            |  | Parts by weight |
|------------------------------------------------------------------------|--|-----------------|
| Titanium dioxide pigment                                               |  | 80              |
| Lead chromate pigment                                                  |  | 16              |
| 65 Dioctyl phthalate plasticizer                                       |  | 136             |
| Polyvinyl chloride resin                                               |  | 410             |
| Mineral spirits                                                        |  | 110             |
| Butylated urea-formaldehyde resin (60% solids in 50-50 butanol-xylene) |  | 13.8            |

Following application of the organosol print paint, the material is fused by passing through infrared lamps or other source of heat.

The floor coverings of my invention are characterized by excellent properties, such as resistance to alkalis, oils, and the like, and are further characterized by resistance to indentation and gouging due to the resistance of the coating paint to the materials contained in the aerosol print paints. While particular reference has been made to floor coverings, the products of my invention may also be employed as a wall covering.

I claim:

1. A plastic floor or wall covering comprising a saturated felt backing, an intermediate seal coat, the binder of which contains about 3% to about 20% by weight of casein and about 97% to about 80% by weight oleoresinous varnish, and a block printed top coat containing a vinyl resin and a plasticizer system having a solvent action on said oleoresinous varnish.
2. A plastic floor or wall covering comprising an asphalt saturated felt backing, an intermediate seal coat, the binder of which contains about 3% to about 20% by weight of casein and about 97% to about 80% by weight oleoresinous varnish, and a block printed top coat containing fused polyvinyl chloride and a plasticizer system having a solvent action on said oleoresinous varnish.
3. In the manufacture of block printed floor or wall

coverings having a saturated felt backing and a fused vinyl resin top coat containing a plasticizer system having a solvent action on oleoresinous varnish, the improvement comprising coating said saturated felt with an intermediate composition, the binder of which contains about 3% to about 20% by weight of casein and about 97% to about 80% by weight oleoresinous varnish.

4. In the manufacture of block printed floor or wall coverings having an asphalt saturated felt backing and a fused polyvinyl chloride resin top coat containing a plasticizer system having a solvent action on oleoresinous varnish, the improvement comprising coating said asphalt saturated felt with an intermediate coat of paint, the binder of which contains about 3% to about 20% casein and about 97% to about 80% by weight oleoresinous varnish.

References Cited in the file of this patent

UNITED STATES PATENTS

|    |           |           |               |
|----|-----------|-----------|---------------|
| 20 | 1,176,853 | Prifold   | Mar. 28, 1916 |
|    | 1,300,043 | Talbert   | Apr. 8, 1919  |
|    | 2,133,886 | Beegle    | Oct. 18, 1938 |
|    | 2,453,052 | Van Etten | Nov. 2, 1948  |
|    | 2,554,899 | Cowgill   | May 29, 1951  |